

July 22, 1952

I. M. LE BARON

2,604,208

PROCESS FOR CONCENTRATING NONMETALLIC MINERALS

Filed Sept. 14, 1948



Fig. 1



Fig. 2



Fig. 3

IRA M. LE BARON  
INVENTOR.

BY Ernest V. Haines  
Attorney

## UNITED STATES PATENT OFFICE

2,604,208

PROCESS FOR CONCENTRATING  
NONMETALLIC MINERALS

Ira M. Le Baron, Lakeland, Fla., assignor to International Minerals & Chemical Corporation, a corporation of New York

Application September 14, 1948, Serial No. 49,192

17 Claims. (Cl. 209—441)

1

The present invention relates to an improved process for the concentration of non-metallic minerals from ore containing the same. More particularly, the invention relates to an improved process in the table concentration of non-metallic ores such as phosphate rock, sylvinitite, and the like.

The art of concentrating non-metallic minerals by both tabling and flotation operations is quite comprehensive and of long standing. By such processes a mineral, in a suitably comminuted state, may be subjected to the action of a riffled table by flowing an aqueous suspension or pulp of the mineral across the surface of said table in a stream of water or brine. The separation of the desired mineral values from the less desirable values or gangue is accomplished due to the inherent specific gravity of the particular minerals present in the ore. The mineral constituents having a lower specific gravity tend to float on the surface of the liquid phase of the suspended ore or pulp. By inclining the surface of the table and flowing the suspended or pulped ore across a riffled surface, the lighter particles tend to flow across the riffles and are collected in a suitable launder. The particles of greater density collect along the leading or feed side of the riffles, thereby achieving a separation of desired minerals from the gangue particles present in the ore. The percent recovery or the extent of up-grading of any particular ore will depend upon the difference in density between the various ore constituents, upon the rate of flow across the riffled table, upon the direction of the riffling, upon the extent to which the surface of the table is inclined, and other factors. In many instances it is desirable to preliminarily reagentize the aqueous mineral suspension or pulped ore prior to the tabling operation. For example, it is common knowledge that suitably comminuted phosphate rock or sylvinitite ore may be pulped in an appropriate aqueous medium to which has been added reagent which will float one component of said ores while the other component will tend to sink when subjected to concentration operations. The pulp may then be subjected to a tabling operation whereby the reagentized ore is flowed in a stream of water over a riffled, inclined surface. The reagentized particles are collected at the lower edge of the table in a launder while the heavier particles collect at the leading edge of the riffles. In most instances, a shaking table is employed in order to continuously remove the heavier particles from the riffles, this being accomplished by

2

the forces imparted to the particles by the shaking action of the table. This will produce a band of heavier particles along the side of the table opposite to the side to which the shaking force is imparted. Such a process is described in Patent No. 1,968,008 issued to Chapman and Littleford, and Patent No. 2,120,535 issued to Wilkinson. According to the teachings of Chapman and Littleford, the finely divided phosphate-bearing material may be reagentized in an aqueous pulp with a suitable amount of a fatty acid or similar reagent and a suitable amount of a non-saponifiable oil. The reagentized pulp is then flowed in a stream of water across a riffled shaking table, thereby achieving the concentration of the phosphate values in the phosphate rock to the extent that the ultimate product which is collected in the concentrate launder has a B.P.L. (bone phosphate of lime) content of about 70%. In a similar manner, it is known that sylvinitite ore may be pulped in an aqueous solution which is substantially saturated with respect to said ore, followed by reagentizing the resultant mixture with a fatty amine type reagent or water-soluble acid addition salts thereof. The reagentized pulp is then flowed in a stream of brine across a riffled shaking table, thereby achieving a concentration of the sylvite (potassium chloride) values contained in the ore. The halite particles collect along the leading edge of the riffles and are removed as tailings in a band along the side of the table opposite to the side to which the shaking force is imparted. It has also been proposed to employ this type of operation for the up-grading or concentration of a middling fraction from a rougher table concentration of either phosphate rock or sylvinitite ore, whereby the desired mineral values contained in such a fraction are further recovered in order to improve the over-all utility of the process. Because of characteristics inherent in the table concentration of minerals by flotation methods, it has been found necessary in several instances to employ a rougher concentration whereby a concentrate, middling fraction, and a tailings fraction are obtained. This is followed by reprocessing the middling fraction on a cleaner table. Due to the fact that the specific gravity of the particular mineral constituents in an ore do not differ sufficiently, a portion of the desired minerals which are being floated in any table operation will ultimately be found in the middling fraction. This is due either to occlusion or to mechanical entrapment 55 of the floatable constituents by the heavier par-

ticles. The middling fraction is usually "dereagentized" by a suitable chemical treatment; followed by a subsequent table concentration of said fraction, in order to improve the over-all recovery of the desired mineral constituents of the ore. Even when such a series of tabling operations is conducted, the tailings or discarded fraction of the ore nevertheless contains a small amount of the desired mineral constituents of the ore; but economic considerations preclude a further recovery of such minerals from said fraction.

It is an object of the invention to provide an improved process for the table concentration of non-metallic minerals from ore containing the same, by flotation methods.

It is a further object of the invention to provide an improved process for the table concentration of non-metallic minerals from ore containing the same, by flotation methods whereby an improvement in the over-all recovery of particular mineral constituents present in said ore is achieved.

It is a further object of the invention to provide an improved process for the table concentration of non-metallic minerals from ore containing the same, by flotation methods whereby a mineral constituent, present in minor amounts in any particular flotation feed, is recovered in good yields.

It is a further object of the invention to provide an improved process for the table concentration of the phosphate values present in phosphatic ore, by flotation methods whereby an improvement in the over-all recovery of said values is achieved.

It is a further object of the invention to provide an improved process for the table concentration of the phosphatic ore, by flotation methods whereby a middlings fraction obtained in a rougher table concentration of phosphate ore, and which contains a major amount of silica and a minor amount of phosphate values, may be so treated as to achieve an improved recovery of the phosphate values contained therein.

It is a further object of the invention to provide an improved process in the table concentration of sylvite ore, by flotation methods whereby improvement in the over-all recovery of either sylvite or halite particles present therein is achieved.

It is a still further object of the invention to provide an improved process for the table concentration of a composition comprising sylvite and halite particles, by flotation methods whereby improved concentrations of the minor constituent of said salts present in the composition may be obtained.

The above objects, as well as others which will become apparent upon a complete understanding of the invention as hereinafter fully described, are accomplished by flowing a reagentized pulp of non-metallic mineral-containing ore, which also contains gangue particles, in a stream of water, brine, or other suitable aqueous medium over a rifled surface while directing a stream of water, brine, or other suitable aqueous medium into the heavier or non-floatable and non-floating particles which are present and collect along the feed side of the riffles; said stream being so positioned that at least one riffle with said stream precedes at least one riffle without said stream with respect to the direction of flow of the feed across the rifled surface. The rifled surface employed as a concentrating device, and the type of concentrating process employed, may be similar to those described in the aforesaid Chapman et al. and

Wilkinson patents; or as described in Section 11, pages 59-60 of a publication by W. A. Taggart, entitled "Handbook of Mineral Dressing," published in 1945. While it is not essential to the operation of the instant process that the rifled surface be placed on an inclined plane during the concentration operation, it has been found to be the preferable practice to incline the plane of the rifled surface so that the feed side of said surface is higher than the concentrate side. For example, it has been found that the feed side of the rifled surface may be advantageously elevated as much as 6-12% with respect to the elevation of the concentrate side of said surface. Furthermore, while it is not essential that the rifled surface employed as a concentrating device in the instant process be subjected to agitative and/or longitudinal motion, it is the preferable practice to employ various devices, which are usually placed at one of the short ends of the table surface, in order to impart a shaking or agitative motion to said surface. Such devices are described in the aforesaid Taggart publication. While the instant process will be described in terms of an inclined, rifled surface which is subjected to longitudinal agitation by means of a shaking device, it is to be understood that other types of rifled surfaces which may or may not be inclined, or of the shaking type, are deemed to be within the scope of the present invention.

Generally speaking, the instant process is carried out by preparing an aqueous pulp of a non-metallic mineral of the type which will be hereinafter described, and reagentizing said pulp with either a cationic or positive-ion agent for the flotation of non-metallic minerals having an affinity for such agents, or employing an anionic or negative-ion agent in the event that mineral constituents having an affinity for such reagents are to be recovered from ores containing the same. It is known to those skilled in the art that usually only about 1%, or a fraction thereof, of such agents will be required for the conditioning of any particular non-metallic mineral-containing pulp. In some instances it is desirable to incorporate into the pulped ore a similar amount of a non-saponifiable oily material which will act as a frothing or co-operating agent and which will assist the reagent in the flotation operation. The reagentized pulp is then subjected to the concentrating action of an inclined, rifled surface of the type previously described by admitting the same through a feed box placed at the upper end of said surface and distributing the pulp through a suitable device along the upper side of said surface. As the pulp flows across the rifled surface due mainly to gravitational force, it is aided by a washing stream of water or brine (as the case may be) which is projected across the riffle surface from the upper end or feed side of the table. Meanwhile, the entire table is subjected to longitudinal agitation by means of a conventional device of the type herein previously described. The reagentized constituents of the ore proceed across the riffles, presumably due to skin flotation, usually in a direction transverse with respect to the movement of the table, and are ultimately collected in a launder or similar device placed at the lower edge of the table. The non-floating and unreacted, non-floatable or gangue constituents of the ore collect along the feed side of the riffles, the greater portion thereof being concentrated along the riffles at the high side of the table. These particles are removed from the table due to the rectilinear motion imparted thereto by

the agitative forces of the table, and are collected in a launder or other suitable device placed at the edge of the table opposite the edge to which the shaking forces are being directed. It has now been found possible to increase the capacity of tabling devices and improve the over-all recovery of any particular mineral constituent of an ore by projecting a stream of water, brine, or other suitable aqueous medium—preferably in the form of jets—into the non-floating and non-floatable particles which are present along the feed side of any particular riffle. The reagentized or floatable particles which are usually occluded or mechanically entrapped therein, due to the inherent characteristics of table concentration, may be removed thereby from their mixture with said non-floatable particles and collected in the launder at the concentrate edge of the table. The streams of liquid media which are jetted into the particles held behind the riffles cause a turbulence of said particles, thereby freeing the reagentized and floatable minerals contained therein. Since this turbulence also causes some of the gangue particles to flow across the riffle along which it has collected, it is essential to the operation of the instant process that at least one riffle which is not equipped with aqueous streams or jets be placed on the low side of the riffle which is equipped with said streams or jets in order that said heavier particles which flow over the riffle equipped with a water stream or jets will not ultimately be collected in the aforesaid launder together with floatable particles. While it is preferable to employ a construction wherein one riffle without a jetted stream is interposed between riffles equipped with said streams, the apparatus may be so constructed that a plurality of riffles without said jetted streams may be positioned between two riffles which are equipped with same.

While the instant process is applicable to the table concentration by flotation methods whereby the desired mineral constituent of said ore is recovered in the concentrate launder, it is particularly adaptable to a tabling operation whereby a middlings fraction obtained in the rougher concentration of a non-metallic mineral ore, in accordance with procedures described in the aforesaid Chapman et al. and Wilkinson patents, may be treated in order to recover the minor but desired mineral constituent of said middlings fraction, while rejecting the major undesired metallic constituents thereof as tailings.

The term "non-metallic minerals," as employed herein and in the appended claims, includes all minerals which are adaptable to the concentration of certain mineral constituents contained therein by the flotation concentration of a reagentized pulp containing said minerals. Such minerals include phosphate rock of the type found in the phosphate areas in Florida and Tennessee; sylvinitic ore such as that found in the Permian Basin, particularly in the Carlsbad, New Mexico area; and bauxite, iron oxide, barytes, lead and zinc carbonates, and similar ores which are amenable to flotation concentration operations. Certain of these minerals—for example, phosphate ore—may be concentrated with negative-ion or anionic reagents such as the high molecular weight fatty acids (oleic, palmitic, stearic and others), resin acids, rosin, tall oil, napthenic acids, and the alkali metal soaps of such materials—for example, the sodium soap of tall oil. Also included in the term "negative-ion agent" are reagents such as

high molecular weight aliphatic alcohol esters—for example, octyl sulfate; high molecular weight xanthates, and the like. Certain other minerals—for example, sylvinitic ore which contains sylvite (KCl) and halite (NaCl) particles—are amenable to concentration by employing either the anionic reagents previously described or cationic reagents such as high molecular weight aliphatic amines—for example, octyl-, hexadecyl-, octadecylamine, etc.—and their salts, with water soluble acids; esters of amine alcohols—for example, oleylethanolamine—and their salts, with water soluble acids; long chain alkyl-substituted isoureas, high molecular weight aliphatic quaternary bases, and their salts, with water soluble acids; and similar reagents. In the case of sylvinitic ore, anionic reagents will float the halite particles while cationic reagents will float the sylvite particles. The instant novel process is adaptable to the table concentration, by flotation methods, of either sylvite or halite from sylvinitic ore.

The instant process will be more fully understood when considered together with the accompanying drawing which discloses, in Figure 1, a more or less diagrammatic plan view of a riffled shaking table device of the type manufactured by the Deister Concentrator Company. Figure 2 is an end, sectional elevation along the line A—A' of Figure 1; and Figure 3 is a longitudinal sectional elevation along the line B—B' of Figure 1. The deck of the table is rhombohedral in shape with a rectilinear motion imparted to the table by means of any suitable shaking device such as an Overstrom head motion device of the type described in the C. P. Taggart publication hereinbefore referred to, Section 11, page 76. The agitative motion imparted to the table by this device is in the direction of the short diagonal of the table. The table is tilted from the horizontal plane to allow feed to flow by gravity from the feed box to the launders. Referring now to Figure 1, riffles 2 and 3 are placed in the direction of the short diagonal and substantially parallel to the rectilinear motion of the table. The riffling of the table is accomplished by placing upon the surface thereof, about one inch apart, cleats 2, made of wood or other suitable material. The height of the cleats will vary from about  $\frac{1}{16}$  inch at the head of the table, and feathering at the tailings end of the table. The small riffles 2 are placed in units of seven or eight, and between each unit is placed a riffle 3 which is slightly higher than the grouped riffles, but which also tapers or feathers towards the tailings end of the table. A non-metallic mineral which has been conditioned with reagent in an aqueous pulp is fed to the table through a feed box 4, and distributed across the upper surface of the table by the distributing box 5. Due to the inclined plane of the table, the reagentized pulp flows across the surface thereof; being aided not only by the agitative motion imparted to the table by means not shown but of the type previously herein described, but also by the assistance of a stream of water or other suitable aqueous media which is admitted to the surface of the table through gate valve 6 and through a distributing device 7. The water flow across various sections of the table is regulated by rotatable wooden diamond-shaped cocks 8. The reagentized particles proceed in the direction of the launder 9 by flowing across the riffles, while the non-floatable gangue particles and other non-floatable con-

stituents of the ore are trapped along the feed side of the riffles and proceed to the right-hand side of the table to launder 10, due to the force imparted to such particles by the agitative motion of the table. The instant process is illustrated by placing pipes 11—which may be constructed of iron, steel, rubber, plastic, or other suitable material—above and across the surface of the table and substantially parallel with respect to the riffles 3. The pipes 11 are supported and supplied with water by conduits 12, and are perforated at suitable intervals so that a plurality of jets of water may be projected into the particles present and collected along any desired length of any particular riffle. Figures 2 and 3 indicate more clearly the positioning of perforated pipes 12 with respect to the riffles 2 and 3, whereby jets of water or other suitable aqueous media are directed into the gangue particles which collect along the feed side of the riffles 3. While the drawings illustrate the position of said pipes above the feed side of the riffles 3 and parallel thereto, it is to be understood that the pipes may be also placed above the feed side of any one of a plurality of riffles, either 2 or 3, providing that at least one riffle without jets is positioned between riffles equipped with jets. It is preferable to conduct the instant process by directing water jets along a riffle by means of a perforated pipe; but it is not intended that the invention be limited to any such particular device. On the contrary, water jets may be projected into the particles collected along any particular riffle or plurality of riffles by employing several lengths of pipe vertically positioned along the feed side of any particular riffle, thereby achieving substantially the same results. Alternatively, a pipe may be horizontally positioned along the feed side of one or more riffles, said pipe being provided with a continuous or discontinuous slot or orifice which faces the surface of the table. Water may then be directed into the gangue particles through said slot, thereby providing a plurality of streams of water which agitate the particles present along the feed side of the riffles and into which said streams are directed.

In a preferred embodiment of the invention, a finely divided phosphate-bearing material, which comprises the middlings fraction of a flotation table concentration of phosphate ore as obtained from a rougher table concentration of phosphate ore in accordance with conventional procedures which have been established in the phosphate industry, and which contains silica and phosphate values in the ratio of about 2 to about 1 parts by weight of silica per part of phosphate, is conditioned in an aqueous pulp with a small amount of anionic or negative-ion agent of the type previously herein described. Preferably, a fraction of 1% of tall oil, or sodium soap thereof, and a small amount of unsaponifiable oil—for example, a fraction of 1% of fuel oil—are employed. The reagentized pulp is then admitted into the feed box of an apparatus similar to that which is diagrammatically described in the accompanying drawing. It is subsequently distributed over the upper edge of the riffled surface and is permitted to flow across the riffled surface in a stream of water which enters the table through a distributor. As a result of the concentrating action of this table, augmented by the water jets which have been incorporated into the device by means of four or five perforated pipes 11 positioned along riffles 75

3, a concentrate is collected in launder 9 which contains about 76% B. P. L. on a dry basis, achieving a recovery of about 90% of the phosphate values present in the feed to the table. This is in contrast with a recovery of about 30% which is achieved by such an operation in the absence of water jets applied to the riffles of a table concentrator.

In a further embodiment of the invention, a composition comprising sylvite and halite present in a ratio of between about 1 and about 2 parts by weight of sylvite per part of halite, and which has been obtained as a combination middlings and tailings fraction from a rougher table concentration of sylvinitic ore in accordance with methods established in the potash industry, is conditioned in a brine which is saturated with respect to sylvite with reagent selected from the group consisting of aliphatic amines containing at least one alkyl group having 7 to 18 carbon atoms and their water-soluble acid addition salts. A particularly high concentration of sylvite may be obtained by conditioning a sylvite-halite composition containing said materials in the aforesaid ratio by conditioning the pulp with reagent consisting of the acetic acid addition salts of a mixture of the aliphatic amines comprising about 25% by weight of hexadecylamine and about 75% by weight of octadecylamine. The resultant reagentized pulp is then fed to a table concentrating device of the type described in the accompanying drawing, which is equipped with brine jets, said brine being substantially saturated with respect to sylvite or sylvinitic. A concentrate of sylvite or potassium chloride is collected in the launder 9, while the halite or sodium chloride values are collected in launder 10 and discarded. An improvement in the over-all recovery of sylvite from sylvinitic ore is obtained which approximates that achieved in the concentration of phosphate values as illustrated by the process described in the preceding paragraph.

In still a further embodiment of the invention, halite may be concentrated from sylvinitic ore, or from compositions containing sylvite and halite, by preparing an aqueous pulp of the material to be concentrated by admixing the same with an aqueous solution which is substantially saturated with respect to halite, and reagentizing the resultant pulp with negative-ion agent having an affinity for halite particles. Preferably, a small amount of composition, comprising agent selected from the group consisting of fatty acids having 7 to 18 carbon atoms, tall oil, rosin, and alkali metal soaps of said agents may be employed in order to properly condition the pulp. The reagentized mixture is then flowed across a device of the type illustrated in the accompanying drawing in a direction transverse with respect to the movement of the agitative motion of the riffled table. Brine jets are directed through four or five pipes 11 positioned along the riffles 3 of the table into the sylvite particles which are present along the feed side of the riffles, said brine being substantially saturated with respect to halite. This achieves an over-all recovery of halite from compositions containing the same in association with sylvite to a degree which has heretofore been impossible to achieve.

In order to more fully illustrate the nature and character of the invention, but with no intention of being limited thereby, the following example is recited:

*Example*

A phosphatic rock typical of the type found in the Florida phosphate area was preliminarily classified to a mesh size of -1 mm. to +35 mesh. This fraction of the rock was then reagentized in an aqueous pulp with about 1.5 lbs. of tall oil, about 2 lbs. of fuel oil, and about 0.5 lb. of kerosene. A sufficient amount of an aqueous solution of caustic soda was added thereto in order to produce a final mixture having a pH between about 8.5 and 9.0. The resultant pulp was then subjected to a rougher concentration for the recovery of the phosphate values contained in the rock by flowing the same over a Deister-Overstrom diagonal table of the type described in the Taggart publication previously mentioned herein and as illustrated diagrammatically in the accompanying drawing. No water jets were used in this particular operation. The rougher table concentration produces three fractions: that is, a concentrate containing about 75% B. P. L., a small tonnage middling fraction which is circulated back to the feed, and a tonnage of rougher tails which is about 20% of the original feed. These rougher tails contain about 25-35% B. P. L. They are then subjected to a second tabling, after re-reagentizing with a small amount of tall oil, fuel oil, and kerosene, plus enough caustic to give the pulp a final pH of about 8.5-9.

The concentrate which is obtained by the tabling of the rougher tails contains about 75-80% B. P. L. and about 2-5% insoluble on a dry basis. The tails from this operation analyzed about 25% B. P. L. with about 68% insoluble. The percent recovery of the phosphate values contained in the feed or rougher tails fraction is about 32%.

During the table concentration of the rougher tails fraction as described above, the concentrating action of the table was augmented by directing water jets into the particles which collect along the feed side of the riffles. This was accomplished by placing perforated pipes along the feed side of four or five of the large riffles 3 and substantially parallel thereto, and forcing water through the perforations into the silica particles. As a result, the concentrate containing the phosphate values has a B. P. L. content of between about 75 and 77%, and an insoluble content of between about 6 and about 8%, on a dry basis. The tailings from this operation have a B. P. L. content of only about 5%, and an insoluble content of about 93%. The recovery of the phosphate values contained in the feed to the table was between about 88 and about 90%, based upon the phosphate values contained in the rougher tailings fraction obtained in the rougher section.

It becomes immediately apparent that nearly a three-fold improvement in the over-all recovery of phosphate values in the feed to the table is obtained by employing water jets in the manner contemplated in the instant process. Also, the B. P. L. content of the tailings has decreased to only about one-fifth of that present in tailings obtained in the absence of the water jet operation. Not only is an improvement in percent achieved, but it is possible to greatly increase the rate of feed to the table, thereby increasing the concentrating capacity of same. The small increase in the percent insolubles present in the concentrate when employing water jets in accordance with the instant process is not deleterious and is amply compensated by the im-

proved recoveries of the phosphate values contained in the feed.

While the above example illustrates the concentration of the phosphate values present in a particular phosphatic-siliceous composition, it is to be understood that other minerals of the type previously herein described may also be advantageously concentrated, attendant with improved recoveries by employing suitable extensions and modifications of the process as above illustrated. It is known that certain reagents are more specific for particular mineral values contained in the various ores which have been mentioned herein; and that the choice of reagents, rate of flow of the flotation feed across the riffled concentrating surface, the angle of inclination of said surface during the concentration, and the degree of agitation will be dependent upon the particular mineral or mineral-containing composition which is sought to be concentrated.

While the example recited herein illustrates the use of a Deister-Overstrom diagonal deck concentrating table, it is to be understood that other types of riffled concentrating surfaces may be employed which may or may not be subjected to agitative motion. For example, the table devices devised by Rettinger, Wilfley, and others, as illustrated in the aforementioned Taggart publication, may also be employed; the choice of any particular device depending upon the mineral to be concentrated from a specific ore.

It is not intended to limit the instant process to the particular procedural details described herein; but any extensions and/or modifications which are equivalent thereto are deemed to be within the scope of the invention.

Having thus fully described the nature and character of the invention, what is desired to be secured by Letters Patent is:

1. In a process for concentrating non-metallic minerals from ore containing the same in association with gangue particles by flowing a reagentized pulp of said ore in an aqueous stream over a riffled surface; the improvement comprising directing an aqueous stream from a point above the table into the particles present along and collected at the feed side of the riffles, at least one riffle with said stream preceding at least one riffle without said stream with respect to the direction of flow of said pulp, and collecting a concentrate of said minerals.

2. In a process for concentrating non-metallic minerals from ore containing the same in association with gangue particles by flowing a reagentized pulp of said ore in an aqueous stream over a riffled surface; the improvement comprising directing a plurality of aqueous jets into the particles present along and collected at the feed side of the riffles, said jets being so positioned that at least one riffle without jets is situated between riffles with jets, and collecting a concentrate of said minerals.

3. In a process for concentrating non-metallic minerals from ore containing the same in association with gangue particles by flowing a reagentized pulp of said ore in an aqueous stream over a riffled, inclined surface; the improvement comprising directing a plurality of aqueous jets from a point above the table into the particles present along and collected at the feed side of the riffles, said jets being so positioned that at least one riffle without jets is situated between riffles with jets, and collecting a concentrate of said minerals.

4. In a process for concentrating non-metallic minerals from ore containing the same in association with gangue particles by flowing a reagentized pulp of said ore in an aqueous stream over a riffled, inclined, moving surface; the improvement comprising directing a plurality of aqueous jets into the particles present along and collected at the feed side of the riffles, said jets being so positioned that at least one riffle without jets is situated between riffles with jets, and collecting a concentrate of said minerals.

5. In a process for concentrating phosphate values from a phosphatic ore containing the same in association with silica by flowing an aqueous reagentized pulp of said ore in a stream of water over a riffled, inclined, moving surface; the improvement comprising directing a plurality of water jets into the particles present along and collected at the feed side of the riffles, said jets being so positioned that at least one riffle without jets is situated between riffles with jets, and collecting a concentrate of phosphate values.

6. In a process for concentrating phosphate values from a phosphatic ore containing the same in association with silica by flowing an aqueous reagentized pulp of said ore in a stream of water over a riffled, inclined, moving surface; the improvement comprising directing a stream of water from a point above the table into the particles present along and collected at the feed side of the riffles, at least one riffle with said stream preceding at least one riffle without said stream, with respect to the direction of flow of said pulp, and collecting a concentrate of phosphate values.

7. In a process for concentrating phosphate values from a phosphatic ore containing the same in association with silica by flowing an aqueous pulp of said ore which contains negative-ion agent having an affinity for phosphate values in a stream of water over a riffled, inclined, moving surface; the improvement comprising directing a plurality of water jets from a point above the table into the particles present along and collected at the feed side of the riffles, said jets being placed at alternate riffles and substantially parallel thereto, and collecting a concentrate of phosphate values.

8. A process for concentrating finely divided phosphate-bearing material containing a major amount of silica and a minor amount of phosphate values, which comprises reagentizing an aqueous pulp of said phosphate-bearing material with negative-ion agent having an affinity for phosphate values; flowing the reagentized pulp in a stream of water over a riffled, inclined, moving surface in a direction transverse with respect to the movement of said surface; directing a plurality of water jets from a point above the table into the particles present along and collected at the feed side of the riffles, said jets being placed at alternate riffles and substantially parallel thereto; and collecting a concentrate of phosphate values.

9. A process for concentrating finely divided phosphate-bearing material containing silica and phosphate values in a ratio of about two to about one parts by weight, which comprises preparing an aqueous pulp of the said phosphate-bearing material; reagentizing said pulp with a small amount of tall oil soap and a small amount of unsaponifiable oil to selectively float the phosphate values; flowing the reagentized pulp in a stream of water over a riffled, inclined, moving surface in a direction transverse with respect to

the movement of said surface; directing a plurality of water jets from a point above the table into the particles present along and collected at the feed side of the riffles, said jets being placed at alternate riffles and substantially parallel thereto; and collecting a concentrate of phosphate values.

10. A process for concentrating finely divided phosphate-bearing material containing silica and phosphate values in a ratio of about two to about one parts by weight, which comprises preparing an aqueous pulp of said phosphate-bearing material; adding thereto a fraction of 1% of sodium soap of tall oil, a fraction of 1% of fuel oil, and a fraction of 1% kerosene; flowing the reagentized pulp in a stream of water over a riffled, inclined, moving surface in a direction transverse with respect to the movement of said surface; directing a plurality of water jets into the particles present along and collected at the feed side of the riffles, said jets being placed at alternate riffles and substantially parallel thereto; and collecting a concentrate of phosphate values.

11. In a process for concentrating sylvite from sylvinitic ore by flowing an aqueous reagentized pulp of said ore in a stream of brine over a riffled, inclined, moving surface; the improvement comprising directing a plurality of brine jets into the particles not floated and which are present along and collected at the feed side of the riffles, said jets being so positioned that at least one riffle without jets is situated between riffles with jets and said brine being substantially saturated with respect to sylvite, and collecting a concentrate of sylvite.

12. In a process for concentrating sylvite from sylvinitic ore by flowing an aqueous reagentized pulp of said ore in a stream of brine over a riffled, inclined, moving surface; the improvement comprising directing a stream of brine into the particles not floated and which are present along and collected at the feed side of the riffles, at least one riffle with said stream preceding at least one riffle without said stream with respect to the direction of flow of said pulp and said brine being substantially saturated with respect to sylvite, and collecting a concentrate of sylvite.

13. In a process for concentrating sylvite from sylvinitic ore by flowing an aqueous pulp comprising finely divided sylvinitic ore, said ore being reagentized with a positive-ion agent having an affinity for sylvite, in a stream of brine over a riffled, inclined, moving surface; the improvement comprising directing a plurality of brine jets into the particles present along and collected at the feed side of the riffles, said jets being placed at alternate riffles and substantially parallel thereto and said brine being substantially saturated with respect to sylvite, and collecting a concentrate of sylvite.

14. A process for concentrating sylvite from a composition comprising sylvite and halite in a ratio of about one to about two parts by weight, which comprises preparing an aqueous pulp of said composition; conditioning the pulp with reagent selected from the group consisting of aliphatic amines containing at least one alkyl group having 7-18 carbon atoms and their water-soluble acid addition salts; flowing the reagentized pulp in a direction transverse with respect to the movement of said surface; directing a plurality of brine jets into the particles present along and collected at the feed side of the riffles, said jets being placed at alternate riffles and sub-

13

stantially parallel thereto and said brine being saturated with respect to sylvite; and collecting a concentrate of sylvite.

15. A process for concentrating a composition comprising sylvite and halite in a ratio of about one to about two parts by weight, which comprises preparing an aqueous pulp of said composition in a saturated solution of same; conditioning the pulp with reagent consisting of the acetic acid addition salts of a mixture of aliphatic amines comprising about 25% by weight of hexadecylamine and about 75% by weight of octadecylamine; flowing the reagentized pulp in a stream of brine over a riffled, inclined, moving surface in a direction transverse with respect to the movement of said surface; directing a plurality of brine jets into the particles present along and collected at the feed side of the riffles, said jets being placed at alternate riffles and substantially parallel thereto and said brine being saturated with respect to sylvite; and collecting a concentrate of sylvite.

16. A process for concentrating a composition comprising sylvite and halite, which comprises preparing an aqueous pulp of said composition in a solution substantially saturated with respect thereto; reagentizing said pulp with negative-ion agent having an affinity for halite particles; flowing the reagentized pulp in a stream of brine over a riffled, inclined, moving surface in a direction transverse with respect to the movement of said surface; directing a plurality of brine jets into the particles present along and collected at the feed side of the riffles, said jets being so posi-

14

tioned that at least one riffle without jets is situated between riffles with jets and said brine being substantially saturated with respect to halite; and collecting a concentrate of halite.

5 17. A process for concentrating sylvinitic ore, comprising preparing an aqueous pulp of said ore in a solution substantially saturated with respect thereto; reagentizing said pulp with a composition comprising an alkali metal soap of an agent selected from the group consisting of fatty acids having 7-18 carbon atoms, tall oil, rosin, and alkali metal soaps of said agents; flowing the reagentized pulp in a stream of brine over a riffled, inclined, moving surface in a direction transverse with respect to the movement of said surface; directing a plurality of brine jets into the particles present along and collected at the feed side of the riffles, said jets being placed at alternate riffles and substantially parallel thereto and said brine being saturated with respect to halite; and collecting a concentrate of halite.

IRA M. LE BARON.

## 25 REFERENCES CITED

The following references are of record in the file of this patent:

## UNITED STATES PATENTS

| 30 | Number    | Name            | Date          |
|----|-----------|-----------------|---------------|
|    | 1,520,451 | Sperry -----    | Dec. 23, 1924 |
|    | 1,956,296 | Martin -----    | Apr. 24, 1934 |
|    | 1,968,008 | Chapman -----   | July 24, 1934 |
|    | 2,287,115 | McCluskey ----- | June 23, 1942 |